# EUROPEAN PATENT SPECIFICATION

(11) **EP 0 548 124 B1**
(45) Date of publication and mention of the grant of the patent: **08.02.1995**
(21) Application number: 91915628.1
(22) Date of filing: 30.08.1991
(51) Int. Cl.: G03C 7/30

(54) **STABILISERS FOR RX DEVELOPERS**
STABILISATOREN FÜR AMPLIFIKATIONSENTWICKLER
AGENTS STABILISANTS POUR REVELATEURS A OXYDOREDUCTION

(30) Priority: 13.09.1990 GB 9020000
(43) Date of publication of application: 30.06.1993
(73) Proprietor: KODAK LIMITED, Hemel Hempstead Hertfordshire HP1 1JY (GB); EASTMAN KODAK COMPANY, Rochester, New York 14650-2201 (US)
(72) Inventor: TANNAHILL, Amanda, Audrey Kodak Limited, Herts. HP1 1JY (GB)
(74) Representative: Daley, Michael John
(86) International application number: EP9101655
(87) International publication number: WO9205471

(56) References cited:
- EP-A- 0 164 760
- DE-A- 2 633 207
- US-A- 4 045 225

## Description

This invention relates to stabilisers for RX developers. Particularly the invention relates to the processing of photographic materials by redox amplification developer systems in order to ameliorate the inherent instability of such solutions.

In photographic colour development processes, and particularly in the RX, redox amplification, process it is desirable to provide colour development materials which degrade only slowly so that they can be used readily in automatic processing.

In the RX, redox amplification, process "normal sensitometry", is produced from low silver chloride laydown coatings having a coating weight of less than 21mg/929cm²(sqft), and preferably about 13mg/929cm²(sqft), by using a combination of a traditional colour developer with an oxidant. Such developer hybrids are inherently unstable since they contain an intimate admixture of the colour developer with an oxidant which is often hydrogen peroxide. This inherent instability restricts the modes of use of the system and makes maintaining good sensitometry quite difficult.

It has been proposed in Organic Chemistry page 867 Sedgewick to use uric or phosphoric acids as stabilisers for hydrogen peroxide per se. Further from Henn & Carpenter, Phot. Sci. Eng. vol 3, page 135, 1959 it is known to use uric acid as a photographic developer.

We have now found that these acids and their functional salts will stabilise oxidants such as peroxide even in the presence of the normal components of a redox amplification developer system, and that the presence of such acids and/or their functional salts has not only the effect of inhibiting the interaction between the colour developer and the stabiliser, thereby to increase the useful life of the developer solutions, but also beneficially effects the development process to enhance the developed quality of the image by markedly reducing the tendance of such systems to produce fogged products.

In a further aspect of the invention it has been found that uric acid, phosphoric acid or its functional salts may be included in a coating on a photographic paper thereby to give improved fogging levels by inhibiting oxidant/colour developer interaction in situ.

In US-A-4,045,225 there is disclosed a colour developer composition comprising an oxidising agent and a colour developing component, wherein the composition additionally comprises a stabiliser such as uric acid for the oxidising agent. However, such composition includes at least one nitro-substituted nitrogen containing hetrocyclic anti-fogging compound. We have now found that the incorporation of a stabiliser such as uric acid into the photographic paper stabilises the development while also acting as an anti-fogging agent thereby enabling said nitrogen containing compound to be dispensed with.

According to the present invention therefore there is provided a redox amplification colour developer composition comprising an oxidizing agent and a colour developing component, characterised in that said composition comprises a combined stabiliser and anti-fogging agent selected from uric acid, phosphoric acid photographically effective salts thereof, but excluding nitro-substituted, nitrogen containing, heterocyclic anti-fogging compounds. It is thus possible to dispense with separate anti-fogging agent per se. The functional salt is preferably an alkali metal salt.

In a preferred form of the invention the composition has a ratio of oxidizing agent to combine stabiliser in the range of 1 ml to 2 to 50 mg of the combined stabiliser, and preferably 1 ml of the agent to 5 - 20 mg of the acid. A preferred concentration of the stabilizer with respect to the developer is 5 to 250mg/l.

According to another aspect of the present invention there is provided a photographic paper suitable for use with a redox amplification colour developer composition, characterised in that the paper incorporates an anti-fogging compound selected from uric acid, phosphoric acid and photographically effective salts thereof; subject to the proviso that the paper does not include nitro-substituted, nitrogen-containing, heterocyclic anti-fogging compounds.

It will thus be seen that an incorporation of the stabilisers in accordance with the present invention inhibit the interaction between the colour developer and the oxidising agent for example hydrogen peroxide thereby increasing the useful lifetimes of solutions for use in automatic processing, while also acting an an anti-fogging agent.

The invention will now be described, by way of illustration only, with reference to the accompanying drawing and with reference to the following example.

The figure annexed hereto shows the graph of the effect of uric acid in amplifying developers.

### EXAMPLE

A multilayer colour paper, suitable for an "RX" process was prepared. The paper was of a similar construction to current 2001 paper products with respect to the dispersions used, and the gel laydown. "All chloride" emulsions were used and the silver concentrations for each layer were as follows - red sensitive layer 3.0mg/929cm²(sqft)., green sensitive layer 4.0mg/929cm² (sqft)., blue sensitive layer 6.4mg/929cm² (sqft), giving a total weight of silver 13.4mg/929cm² (sqft).

An initial developer was prepared using a potassium carbonate buffer, to which the required photographic reagents were added. Final developer composition is shown below.

Key:
- EDTA: ethylene diamine tetracetic acid
- CD3: β-methanesulphonamidoethylaminotoluidine sesquisulphate hydrate

The pH was adjusted to 10.3, with dilute NaOH, or H₂SO₄ as required.

Samples of developer above were then prepared with different concentrations of uric acid. Uric Acid was first dissolved in an alkali solution of KoH, (0.5g K OH plus 0.5g uric acid in 50mls H₂O). Subsequently this solution was used to give developers with various concentrations of uric acid: 0, 25, 50, & 100 mg uric acid/litre of developer.

Control samples of these developers were then taken, whilst the remaining volume was equilibrated to 35°C in a tank line. Hydrogen Peroxide (100 vol.) was added to each developer, to give an oxidant concentration of 5ml/l of developer. Next, suitably exposed sensitometric strips were processed through each of the four experimental developers at intervals over a period of 2.5 hrs. Processing was 30 secs. development, followed by 30 secs. fix, and 90 secs. wash. After each strip samples of the developers were taken for CD3 analysis.

The figure shows a graph of the data from CD3 analysis, clearly the developers with higher uric acid concentrations have more CD3 left than the control sample.

The sensitometric effects of incorporating uric acid into amplifying developers is summarised below, whilst relevant data is given in Tables 1 to 4.

Red & Green D mins both show a relative increase compared to the control. The highest uric acid concentration shows the most stabilising effect.

Blue D min is improved by the incorporation of uric acid in the amplifying developer, the improvement is best at the higher concentrations and is maintained over the test period.

All three D max densities are improved compared to the control by the incorporation of uric acid in the developer and show reduced variations.

Contrasts for the layers show variation, but the magnitude of the uric acid containing samples are reduced compared to the control which is an advantage.

## Claims

1. A redox amplification colour developer composition comprising an oxidising agent and a colour developing component; characterised in that the composition comprises a combined anti-fogging agent and stabiliser for the oxidising agent selected from uric acid, phosphoric acid and photographically effective salts thereof, but excluding nitro-substituted, nitrogen-containing, heterocyclic anti-fogging compounds.

2. A composition according to claim 1 characterised in that the ratio of the oxidising agent to the combined stabiliser is 1 ml to 2 - 50 mg of the stabiliser.

3. A composition according to claim 3 characterised in that the ratio is 1 ml to 5 - 20 mg of the combined stabiliser.

4. A composition according to claim 1 characterised in that the oxidising agent is hydrogen peroxide.

5. A composition according to any preceding claim characterised in that the photographically effective salt is an alkali metal salt.

6. A method of stabilising a redox amplification colour developer composition comprising an oxidising agent and a colour developing component, characterised by adding to the composition a combined stabiliser and anti-fogging compound selected from uric acid, phosphoric acid and photographically effective salts thereof, but excluding nitro-substituted, nitrogen-containing, heterocyclic anti-fogging compounds.

7. A method as claimed in claim 6 characterised in that the oxidising agent is hydrogen peroxide.

8. A method according to claim 6 or 7 characterised in that the concentration of the combined stabilizer with respect to the developer composition is 5 to 250 mg/l.

9. A photographic paper suitable for use with a redox amplification colour developer composition, characterised in that the paper incorporates an anti-fogging compound selected from uric acid, phosphoric acid and photographically effective salts thereof; thereby to inhibit fogging due to interaction between an oxidizing agent a colour developing component on developing the paper; subject to the proviso that the paper does not include nitro-substituted, nitrogen-containing, hetercyclic anti-fogging compounds.

## Patentansprüche

1. Redoxverstärkungs-Farbentwicklerzusammensetzung mit einem Oxidationsmittel und einer Farbentwicklerkomponente,
**dadurch gekennzeichnet**,
daß die Zusammensetzung kombiniert ein Anti-Schleiermittel und einen Stabilisator für das Oxidationsmittel, das unter Harnsäure, Phosphorsäure und ihren photographisch wirksamen Salzen ausgewählt ist, enthält, wobei nitrosubstituierte Stickstoff enthaltende heterocyclische Anti-Schleierverbindungen ausgenommen sind.

2. Zusammensetzung gemäß Anspruch 1, **dadurch gekennzeichnet**, daß das Verhältnis von Oxidationsmittel zu kombiniertem Stabilisator 1 ml auf 2 bis 50 mg Stabilisator beträgt.

3. Zusammensetzung gemäß Anspruch 3, **dadurch gekennzeichnet**, daß das Verhältnis 1 ml auf 5 bis 20 mg des kombinierten Stabilisators beträgt.

4. Zusammensetzung gemäß Anspruch 1, **dadurch gekennzeichnet**, daß das Oxidationsmittel Wasserstoffperoxid ist.

5. Zusammensetzung gemäß einem der vorhergehenden Ansprüche, **dadurch gekennzeichnet**, daß das photographisch wirksame Salz ein Alkalimetallsalz ist.

6. Verfahren zur Stabilisierung einer Redoxverstärkungs-Farbentwicklerzusammensetzung mit einem Oxidationsmittel und einer Farbentwicklerkomponente,
**gekennzeichnet durch**
Zusatz eines kombinierten Stabilisators und einer Anti-Schleierverbindung zur Zusammensetzung, die unter Harnsäure, Phosphorsäure und deren photographisch wirksamen Salzen ausgewählt sind, wobei nitrosubstituierte Stickstoff enthaltende heterocyclische Anti-Schleierverbindungen ausgenommen sind.

7. Verfahren gemäß Anspruch 6, **dadurch gekennzeichnet**, daß das Oxidationsmittel Wasserstoffperoxid ist.

8. Verfahren gemäß Anspruch 6 oder 7, **dadurch gekennzeichnet**, daß die Konzentration des kombinierten Stabilisators, bezogen auf die Entwicklerzusammensetzung 5 bis 250 mg/l beträgt.

9. Photopapier zur Verwendung mit einer Redoxverstärkungs-Farbentwicklerzusammensetzung, **dadurch gekennzeichnet**, daß das Papier eine Anti-Schleierverbindung enthält, die unter Harnsäure, Phosphorsäure und deren photographisch wirksamen Salzen ausgewählt ist, zur Verhinderung einer Schleierbildung infolge der Wechselwirkung zwischen einem Oxidationsmittel und einer Farbentwicklerkomponente bei der Entwicklung des Papiers, mit der Maßgabe, daß das Papier keine nitrosubstituierten Stickstoff enthaltenden heterocyclischen Anti-Schleierverbindungen enthält.

## Revendications

1. Composition de révélateur couleur à oxydoréduction comprenant un agent oxydant et un composant révélateur couleur, caractérisée en ce qu'elle comprend un agent combiné anti-voile et stabilisant pour l'agent oxydant choisi parmi l'acide urique, l'acide phosphorique et leurs sels efficaces photographiquement, mais excluant les composés anti-voile hétérocycles, contenant de l'azote, nitro-substitués.

2. Composition selon la revendication 1, caractérisée en ce que le rapport entre l'agent oxydant et le stabilisant combiné est de 1 ml à 2 - 50 mg du stabilisant.

3. Composition selon la revendication 2, caractérisée en ce que le rapport est de 1 ml à 5 - 20 mg du stabilisant combiné.

4. Composition selon la revendication 1, caractérisée en ce que l'agent oxydant est du peroxyde d'hydrogène.

5. Composition selon l'une quelconque des revendications précédentes, caractérisée en ce que le sel efficace photographiquement est un sel des métaux alcalins.

6. Procédé de stabilisation d'une composition de révélateur couleur à oxydoréduction comprenant un agent oxydant et un composant révélateur couleur, caractérisé par l'addition à la composition d'un stabilisant combiné et d'un composé anti-voile choisi parmi l'acide urique, l'acide phosphorique et leurs sels efficaces photographiquement, mais excluant les composés anti-voile hétérocycles, contenant de l'azote, nitro-substitués.

7. Procédé selon la revendication 6, caractérisé en ce que l'agent oxydant est du peroxyde d'hydrogène.

8. Procédé selon la revendication 6 ou 7, caractérisé en ce que la concentration du stabilisant combiné par rapport à la composition du révélateur est de 5 à 250 mg/l.

9. Papier photographique convenant à l'utilisation avec une composition de révélateur couleur par oxydoréduction, caractérisé en ce que le papier comprend un composé anti-voile choisi parmi l'acide urique, l'acide phosphorique et leurs sels photographiquement efficaces, inhibant ainsi le voile dû à l'interaction entre un agent oxydant, un composé révélateur couleur lors du développement du papier, sous réserve que le papier n'incorpore pas de composés anti-voile hétérocycles, contenant de l'azote, nitro-substitués.
